

1

3,138,456

### CHROMIUM-TANTALUM ALLOYS

Alan R. Edwards, Surrey Hills, Victoria, Australia, assignor to Commonwealth of Australia, Canberra, Australian Capital Territory, Commonwealth of Australia  
No Drawing. Filed May 2, 1960, Ser. No. 25,860  
Claims priority, application Australia Oct. 22, 1956  
6 Claims. (Cl. 75—176)

This invention relates to chromium-tantalum alloys and has for its object the provision of new alloys having good structural properties at high temperatures and particularly suitable for such applications as high performance gas turbine rotor blading.

2

However, the ability to be worked by extrusion, forging, rolling and like procedures is frequently required in alloys for turbine rotor blading and this ability is in general possessed by the alloys of the present invention.

It has been ascertained that alloys containing 0.5 to 7% by weight of tantalum with the balance chromium have satisfactory properties for the purpose of this invention. The amount of tantalum in the alloys is preferably in the range 1 to 4%. At temperatures of 950° to 1000° C. alloys within the range specified have shown minimum creep rates under stress which compare favourably with the creep rates under similar conditions of a high strength heat resistant alloy at present in commercial use as shown in Table I which now follows:

Table I

| Alloy                                         | Condition          | Stress<br>(in tons/<br>sq. in.) | Test<br>Tempera-<br>ture<br>(in ° C.) | Minimum<br>creep rate<br>(in./in./hr.) | Tertiary<br>creep<br>after<br>(hrs.) |
|-----------------------------------------------|--------------------|---------------------------------|---------------------------------------|----------------------------------------|--------------------------------------|
| Commercial high strength heat resistant alloy | Fully heat treated | 6                               | 950                                   | $120-150 \times 10^{-6}$               | 20-21                                |
|                                               |                    | 12                              | 950                                   | $1,600 \times 10^{-6}$                 | 2½                                   |
| Chromium, 1.5% tantalum                       | Extruded           | 6                               | 950                                   | $40 \times 10^{-6}$                    | 1200                                 |
| Chromium, 2% tantalum                         | Cast               | 6                               | 1,000                                 | $7.6 \times 10^{-6}$                   | 1240                                 |
| Chromium, 5% tantalum                         | Forged             | 6                               | 950                                   | $109 \times 10^{-6}$                   | 1126                                 |
|                                               | Cast               | 6                               | 950                                   | Less than $1 \times 10^{-6}$           | 1200                                 |
|                                               | Forged             | 12                              | 950                                   | $12 \times 10^{-6}$                    | 1200                                 |

<sup>1</sup> Test discontinued. No tertiary creep.

Alloys according to the invention are broadly characterized in that they consist essentially of 0.5 to 7% by weight of tantalum, incidental ingredients and impurities including gaseous impurities, iron and other metals not exceeding a total of 0.5%, and the balance chromium.

The term "incidental ingredients and impurities" does not include the metals titanium, vanadium, niobium, molybdenum, aluminum silicon and mixtures thereof, which may be included as a further alloying component, provided that the chromium content should not be less than 85%.

The lower limit of 85% of the chromium content has been found necessary to ensure that the alloys meet the following requirements for gas turbine rotor blading:

(a) *An acceptably low density.*—The tensile stress on rotor blading is directly proportional to the density of the alloy used, so that the accepted density for currently used turbine alloys is substantially less than 9 grammes/cc. To meet this requirement, alloys of chromium with heavy metals must contain not less than 85% chromium.

(b) *Good resistance to high temperature oxidation.*—The naturally high oxidation-resistance of chromium is seriously impaired if it is alloyed with a total of more than 15% of poorly oxidation-resistant heavy metals.

(c) *Acceptable hardness and machineability.*—Alloys of chromium with heavy metals containing less than 85% chromium come into the category of "hard metals," noted for their resistance to wear and to machining operations. It has, however, been ascertained that the alloys of the present invention, containing not less than 85% chromium, can be readily machined with normal machine tools. Since the alloys are required to be finished to the close tolerances of turbine rotor blading, this easy machineability is an essential feature.

(d) *Formability.*—No high-strength alloy which consists preponderantly of chromium with the addition of heavy metals can be formed by the accepted metalworking operations unless it contains at least 85% chromium.

The commercial alloy referred in the foregoing Table I is an alloy of 20% chromium, 16% cobalt, 3% titanium, 2% aluminum and the balance nickel. The expression "Fully heat treated" in the foregoing Table I means "Solution treated 1150° C., and aged 700° C."

The commercial alloy tested had a minimum creep rate of approximately  $1 \times 10^{-6}$ /hr. under a stress of 6 tons/sq. in. at a temperature of 815° C. so that the alloys of the invention provide an advance of up to 140° C. on the existing alloy. On a weight comparison, all the chromium-tantalum alloys of this invention are lighter than the comparison alloy.

Alloys according to the invention can be hot-worked at high temperatures while a proportion of the alloys can be cold worked at lower temperatures.

For hot-working, high speed extrusion is employed, preferably using uncooled steel dies and a molten glass lubricant. The alloy is heated for extrusion in a protective atmosphere of hydrogen or an inert gas, such as argon or helium to minimize surface contamination by atmospheric gases, particularly nitrogen. This heating method is also used for hammer forging, which is conducted in the same temperature range. It is possible to produce a considerable range of shapes by hot-working. In particular, the extrusion method can be used to make aerofoil sections, with or without thickened root sections, suitable for the production of turbine blades.

Thus it has been found possible to extrude the 2% tantalum alloy at temperatures above 1200° C. starting with a 1½" diameter arc-cast ingot and finishing with a ½" diameter rod. Small arc-cast ingots containing up to 5% tantalum can be hammer-forged at temperatures above 1200° C. to a useful extent using particular handling techniques and one blow per heat. The main feature of the handling techniques is the use of tongs and holders made of solid molybdenum. These usually remain in contact with the chromium alloy ingots during the whole of the period of heating prior to forging, thus minimizing the heat loss which would otherwise occur

in transferring the ingots from the furnace to the hammer face.

The strength at high temperature of alloys according to the invention is such that cold-working must usually be conducted at temperatures well above room-temperature, in the range 500°-1300° C.

Heat treatment, if employed, consists of an ageing treatment from 5 to 50 hours at the intended service temperature, or up to 200° C. above this temperature. The normal range for this treatment is 900° C. to 1200° C. This may or may not be preceded by a high-temperature solution treatment in the range 1200° to 1600° C.

The alloys according to the invention may be used in the cast condition, or in the hot-worked or cold-worked conditions, with or without heat-treatment. The materials are intended primarily for the rotor and stator blading of gas turbine engines, and in other applications requiring high load-carrying ability at temperatures of 900° C. and higher.

The alloys can be shaped by normal machining methods, using high-speed steel or carbide tools, or grinding wheels with a copious supply of cutting lubricant.

In addition to tantalum there may be included in the alloys from 0.1 to 7% of one or more of the following elements: titanium, vanadium, niobium, molybdenum, aluminium and silicon. The partial substitution of one or more of these elements for the high-density main alloying addition tantalum gives a desirable reduction in the density of the alloys and it has been ascertained that such substitution causes little or no detriment to the general level of high temperature strength, as shown in Table II which now follows:

Table II

| Alloy                                                                | Condition     | Stress (in tons/sq.in.) | Test Temperature (in ° C.) | Minimum Creep rate (in./in./hr.) | Tertiary creep after (hrs.) |
|----------------------------------------------------------------------|---------------|-------------------------|----------------------------|----------------------------------|-----------------------------|
| Chromium, 3% tantalum, 0.2% titanium, 0.5% silicon.                  | Cast-----     | 6                       | 1,000                      | 19.6×10 <sup>-6</sup>            | 1 330                       |
| Chromium, 2% tantalum, 0.1% titanium, 0.5% silicon.                  | Cast-----     | 6                       | 1,000                      | 13.2×10 <sup>-6</sup>            | 1 243                       |
| Chromium, 2% tantalum, 0.5% niobium, 0.5% silicon.                   | Extruded----- | 6                       | 1,000                      | 51×10 <sup>-6</sup>              | 1 332                       |
| Chromium, 0.5% tantalum, 3% molybdenum, 0.5% titanium, 0.5% silicon. | Cast-----     | 6                       | 1,000                      | 4.4×10 <sup>-6</sup>             | 1 342                       |
| Chromium, 0.5% tantalum, 3% molybdenum, 0.5% titanium, 0.5% silicon. | Cast-----     | 6                       | 1,000                      | 16×10 <sup>-6</sup>              | 1 248                       |

<sup>1</sup> See footnote 1, Table I.

It has further been ascertained that titanium and niobium enhance ductility and general handling qualities and that aluminium and silicon improve the already high oxidation resistance of the alloys, as shown in Table III which now follows:

Table III

| Alloy                                          | Condition           | Weight of oxide scale formed on alloy surface at 1,000° C. (in micro-grammes/sq. cm.) |                |
|------------------------------------------------|---------------------|---------------------------------------------------------------------------------------|----------------|
|                                                |                     | After 7.5 hours                                                                       | After 25 hours |
| Commercial high strength heat resistant alloy. | Fully heat treated. | 604                                                                                   | 1,080          |
| Chromium, 2% tantalum-----                     | Cast-----           | 551                                                                                   | 1,075          |
| Chromium, 2% tantalum, 0.5% silicon.           | Cast-----           | 363                                                                                   | 645            |
| Chromium, 2% tantalum, 2% aluminum.            | Cast-----           | 410                                                                                   | -----          |

The commercial alloy referred to in the foregoing Table III is an alloy of the same composition as the commercial alloy referred to in Table I. These more complex alloys also contain not less than 85% by weight of chromium. They retain the required properties of acceptable hardness, machineability and formability and thus have fully satisfactory properties for the purpose of this invention. There may also be impurities in the alloys,

totalling not more than 0.5%, this total including gaseous impurities such as nitrogen and oxygen and non-gaseous impurities such as iron.

A high strength, heat-resistant alloy falling within the scope of the present invention consists essentially of 0.5 to 4% tantalum, 0.1 to 4% molybdenum, 0.1 to 1% niobium and 0.1 to 2% silicon, incidental impurities including gaseous impurities, iron and other metals not exceeding a total of 0.5%, and the balance chromium. This application contains subject matter common to, and is a continuation-in-part of my patent application Serial No. 850,523, filed November 3, 1959, which latter application, in turn, was a continuation-in-part of my parent patent application Serial No. 690,891, filed October 18, 1957. Applications Serial Nos. 690,891 and 850,523 have since become abandoned.

I claim:

1. A high strength heat resistant alloy consisting essentially of 0.5 to 7% by weight of tantalum, incidental ingredients and impurities including gaseous impurities and iron not exceeding a total of 0.5% and the balance chromium.

2. A high strength heat resistant alloy consisting essentially of 0.5 to 7% tantalum, 0.1 to 7% of a further alloying component selected from the group consisting of titanium, vanadium, niobium, molybdenum, aluminium, silicon and mixtures thereof, and the balance chromium and incidental impurities, the chromium content amounting to not less than 85% by weight of the total alloy composition, and the impurities including gaseous impurities and iron not exceeding a total of 0.5%.

3. A high strength heat resistant alloy consisting essen-

tially of 0.5 to 4% tantalum, 0.1 to 1% titanium and 0.1 to 2% silicon, incidental impurities including gaseous impurities and iron not exceeding a total of 0.5%, and the balance chromium.

4. A high strength heat resistant alloy consisting essentially of 0.5 to 4% tantalum, 0.1 to 4% molybdenum, 0.1 to 1% titanium and 0.1 to 2% silicon, incidental impurities including gaseous impurities and iron not exceeding a total of 0.5%, and the balance chromium.

5. A high strength heat resistant alloy consisting essentially of 0.5 to 4% tantalum, 0.1 to 1% niobium and 0.1 to 2% silicon, incidental impurities including gaseous impurities and iron not exceeding a total of 0.5%, and the balance chromium.

6. A high strength heat resistant alloy consisting essentially of 0.5 to 4% tantalum, 0.1 to 4% molybdenum, 0.1 to 1% niobium and 0.1 to 2% silicon, incidental impurities including gaseous impurities and iron not exceeding a total of 0.5%, and the balance chromium.

#### References Cited in the file of this patent

#### UNITED STATES PATENTS

70 3,030,206 Buck ----- Apr. 17, 1962

#### OTHER REFERENCES

Kubaschewski et al.: Journal of the Institute of Metals, volume 75, 1949, pages 403 and 410-412. Published by the Institute, London, England.